

## 1

2,842,471

POWDER METALLURGY AND PISTON RINGS  
OBTAINED THEREBYMax Koehler, Witten-Bommern, Germany, assignor to  
August H. Schilling, Atherton, Calif.No Drawing. Original application December 22, 1950,  
Serial No. 202,395, now Patent No. 2,741,827, dated  
April 17, 1956. Divided and this application April 2,  
1956, Serial No. 575,687

11 Claims. (Cl. 148—12)

The present invention relates to the manufacture of piston rings for high speed internal combustion engines based upon the pressing and sintering of mixtures of metallic powders, the main ingredient of which is powdered iron, and containing minor proportions of powdered lead and graphite.

The present application is a division of my copending application Serial No. 202,395, filed December 22, 1950, now Patent No. 2,741,827, granted April 17, 1956.

In the known production of objects, for example, piston rings, by the powder metallurgical process, the metal powder is usually subjected to a pressing with a subsequent sintering, that is, a heat treatment wherein the temperature lies considerably under the melting point of the powdered metal mixture. In this type of manufacture, it is well known that the strength of the thus produced sintered body can be increased by the addition of small percentages of manganese, chromium or silicon to the soft iron powder. It has also been attempted to increase the strength of the resultant material by cold-pressing the same subsequent to the sintering or by subjecting it to several sintering treatments. No noteworthy increase in the material strength has, however, been attained by these processes.

It is also known that objects may be made from mixtures of powdered metals when the pressing and sintering processes are combined into a single process of hot-pressing.

Experience has shown, however, that piston rings manufactured according to the above suggestions are not entirely satisfactory for use in high speed internal combustion engines, for the latter impose very high thermal and mechanical stresses upon the rings.

It is the general object of the present invention to provide an improved process for the manufacture of piston rings and other parts for use in engines operating at high speed and at high temperatures.

More specifically, it is an object of the invention to provide an improved process whereby a material suitable for the manufacture of piston rings for high speed internal combustion engines is obtained and in which the crystal structure can be controlled by suitable modifications of the process.

It is a further object of the invention to provide an improved process for the manufacture of piston ring material by powder metallurgy wherein a mixture containing from 1% to 10% of lead with or without other heavy metals, and silicon components all in powdered condition in admixture with powdered iron and a small proportion of powdered graphite, is converted into an extremely strong and heat resistant body, having exceptional bearing qualities, by sintering and pressing, and in such manner that the material is given a lamellar-pearlitic or a granular-pearlitic or sorbitic structure.

Other objects and advantages of the invention will appear more fully from the following more detailed description thereof.

According to the present invention, powdered iron is

## 2

briquetted or preliminarily pressed to approximately the desired final shape after mixing with a small proportion of powdered graphite and with from 1% to 10% of powdered lead which may be replaced in part with one or more other heavy metals (i. e., metals having an atomic weight above 50), with or without silicon, until the specific gravity of the mass is about 6.3 to 6.5. This mass is then sintered at a temperature of about 1000° to 1200° C., depending upon the fusion point of the added metal or metals, for a period of about one to two hours. The mass is then cooled and subjected to cold-pressing at high pressures, and thereafter is brought to a temperature in the range of about 850° to 1000° C., i. e., above the transition or transformation temperature, but no higher than the sintering temperature, after which it is either rapidly quenched, where the material is to be subjected in use to temperatures up to about 300° C., under load, or is allowed to cool slowly where it is to be subjected to maximum temperatures of about 200° C. under load.

When additions of the heavy metals, such as tin, antimony, manganese, chromium, nickel and copper, and also of silicon, are used along with the lead, the ratio of the additions to the quantity of lead must be so regulated that the diffusion processes internal to the mixed crystalline series structure, like Fe—Pb—Sn, Fe—Pb—Si, and Fe—Pb—Sb—Si, are prevented.

My improved process may be varied in several ways for controlling the properties of the final product. In one modification of my process, it is sought to obtain a granular pearlitic or sorbitic structure which is particularly desirable for piston rings subject to high thermal stress in high-load, high-speed internal combustion engines, for example, those in which the operating piston ring temperature reaches approximately 300° C. In a modified procedure, it is desired to attain a fine lamellar pearlitic structure which is particularly desirable for the piston rings of high speed internal combustion engines which are operated at a thermally lower stress, where the ring temperatures do not exceed approximately 200° C.

The lamellar pearlitic structure is attained when, in the production of the piston ring material, iron powder containing a small proportion of graphite is mixed with a heavy metal powder consisting entirely or preponderantly of lead, with or without silicon, in the limits of 1 to 10%, preferably about 5%, which mixture is first pressed to a specific gravity of approximately 6.3 to 6.5 and the briquette is then sintered for from one to two hours at 1000° to 1200° C. followed by a step-wise cold-pressing to a final pressure of about 140,000 lbs./in.<sup>2</sup> (10,000 kg./cm.<sup>2</sup>) to a specific weight of 7.6 to 7.7 and with a final heating to 850° to 900° C. for approximately one hour, followed by a slow cooling. This lamellar pearlitic structure is particularly desirable for piston rings for high speed internal combustion engines operating under thermal stresses of the order of approximately 200° C.

For piston rings for high speed internal combustion engines with thermally more highly stressed rings, for example, where the piston ring operating temperature is approximately 300° C., the following manufacturing procedure will give the desirable granular pearlitic or sorbitic structure to the piston ring material.

The above-mentioned mixture is first consolidated to a specific gravity of 6.3 to 6.5, then sintered for one to two hours at 1000° to 1200° C. and, to obtain a material with a granular pearlitic structure, the briquetting and sintering are followed by a step-wise cold-pressing to about 140,000 lbs./in.<sup>2</sup> by which a specific gravity of 7.6 to 7.7 is obtained. After a subsequent heat treatment at 850° to 900° C. for approximately one hour, a rapid quenching is carried out, for example, in oil.

This last described process can be altered in that the cold-pressing occurs in stages up to pressures of about 210,000 lbs./in.<sup>2</sup> (15,000 kg./cm.<sup>2</sup>) and that after a rapid quenching from approximately 760° to 820°, for example, 800° C., a further soaking occurs at a temperature from 500° to 650° C., or at any temperatures lying under the transition point of approximately 720° C. In further explanation, the following may be noted:

During the cold-pressing, the cementite as well as the free graphite still present, and the mixed crystals of the Fe-C-heavy metal group, which were formed by the sintering subsequent to the briquetting, are distributed. In consequence, a rapid conversion into martensite is obtained by the subsequent heating to 760° to 820° C. with the rapid quenching that follows. With the subsequent soaking at temperatures of approximately 650° C., a grain structure build-up results whose special characteristic is annealed sorbite. This gives to the material the characteristics which are valuable for piston rings; namely, a higher elastic limit, strength and a springiness as well as extremely good running and slipping characteristics as yet not attained by any other process. The length of time required by the soaking must be determined by the cross section of the material and the desired strength; the time increases with larger cross sections and for the reaching of higher strengths.

The following example will serve to illustrate the invention more specifically without, however, indicating the limits thereof.

*Example*

The following materials were mixed together:

|                                                                      | Percent |
|----------------------------------------------------------------------|---------|
| Powdered iron (with impurities of 1%)                                | 94      |
| Powdered graphite (ash content 15%)                                  | 1.5     |
| Powdered lead with additives                                         | 4.5     |
| which mixture had the following approximate grain size distribution: |         |
|                                                                      | Percent |
| Under 0.06 mm                                                        | 20      |
| Between 0.06 and 0.1 mm                                              | 39      |
| Between 0.1 and 0.2 mm                                               | 26      |
| Over 0.2 mm                                                          | 15      |

The initial pressing or briquetting of this material occurred at a pressure of about 70,000 lbs./in.<sup>2</sup> (4,900 kg./cm.<sup>2</sup>) followed by sintering at approximately 1100° C. for two hours in a neutral furnace atmosphere. This crude sintered mass had a porosity of approximately 23% and an ultimate strength of 14,000 to 17,000 lbs./in.<sup>2</sup> (10 to 12 kg./mm.<sup>2</sup>).

After sintering, the mass was cold-pressed in stages until a maximum pressure of about 140,000 lbs./in.<sup>2</sup> (9,800 kg./cm.<sup>2</sup>) was reached. This material was subsequently heated and held for one hour at a temperature of 850° C. (The effect attained by this heating may be developed in a shorter time by the use of a higher temperature, which temperature, however, may not exceed the sintering temperature.) At the end of this annealing, the material was oil-quenched and soaked at a temperature of 650° C. Examination showed it had a definite grainy pearlitic structure, and the characteristics tabulated below:

Elastic limit, kg./mm.<sup>2</sup> 62.6 (89,000 lbs./in.<sup>2</sup>).

Ultimate strength, kg./mm.<sup>2</sup> 74.5 (106,000 lbs./in.<sup>2</sup>).

Elongation 2.

Chemical analysis:

|    |                               |
|----|-------------------------------|
| C  | 0.52%                         |
| Si | 0.16%                         |
| Mn | 0.19%                         |
| P  | 0.003%                        |
| Pb | 3.45%                         |
| Sn | 0.36%                         |
| Cu | 0.52%                         |
| Fe | Remainder<br>(approx. 94.7%). |

While in the foregoing, I have referred specifically to iron as the ferrous component, it will be understood that various suitable types of steel can be employed, in place of various forms of iron, suitable adjustment of the quantity of graphite being made where necessary.

The term "heavy metal" or "heavy metal powder" as employed in the specification and claims is to be understood as having reference to a solid metal of an atomic weight above 50 and of the type commonly employed in the metallurgy of iron and steel, and in minor proportions with reference to the iron, in order to modify the properties of the essentially ferrous product. The lead, tin, antimony, manganese, chromium, nickel, and copper referred to hereinabove are typical examples of additions in modified iron and steel products and ferrous alloys.

I claim:

1. Process for the manufacture of piston rings suitable for use in high speed internal combustion engines, the steps which comprise pressing a mixture of a preponderating proportion of iron powder, about 1 to 10% of lead powder, and a small proportion of powdered graphite to approximately the desired shape, sintering the mass, subsequently cold-pressing the same, and thereafter reheating the pressed mass.

2. Process according to claim 1, wherein the sintering takes place at a temperature of about 1000° to 1200° C. for about one to two hours.

3. Process according to claim 1, wherein the mass is slowly cooled after the reheating.

4. Process according to claim 1, wherein the mass is quenched after the reheating.

5. Process according to claim 4, wherein the sintering takes place at a temperature of about 1000° to 1200° C. for about one to two hours, and wherein the reheating occurs to a temperature above the transformation temperature, but no higher than the sintering temperature.

6. Process for the manufacture of piston rings suitable for use in high speed internal combustion engines, the steps which comprise pressing a mixture of a preponderating proportion of iron powder, about 1 to 10% of lead powder, and a small proportion of powdered graphite to a specific gravity of 6.3 to 6.5, sintering the mass at a temperature of about 1000° to 1200° C. for about one to two hours, subsequently cold-pressing the mass in stages at pressures up to about 140,000 lbs./in.<sup>2</sup> to a specific gravity of 7.6 to 7.7, reheating the mass to a temperature above the transformation point but below the sintering temperature, and then rapidly quenching it.

7. Process for the manufacture of piston rings suitable for use in high speed internal combustion engines, the steps which comprise pressing a mixture of a preponderating proportion of iron powder, about 1% to 10% of lead powder, and a small proportion of powdered graphite to a specific gravity of 6.3 to 6.5, sintering the mass at a temperature of about 1000° to 1200° C. for about one to two hours, subsequently cold-pressing the mass in stages at pressures up to about 210,000 lbs./in.<sup>2</sup>, reheating the mass to a temperature above the transformation point but no higher than the sintering temperature, rapidly quenching the mass, and then annealing the mass at a temperature below the transformation point.

8. In a process for the manufacture of piston rings suitable for use in high speed internal combustion engines, the steps which comprise mixing a preponderating proportion of iron powder with about 1% to 10% of powdered lead and a small proportion of powdered graphite, pressing the mixture to a specific gravity of approximately 6.3 to 6.5, sintering the shaped mass at about 1000° to 1200° C. for about one to two hours, subjecting the mass to a stage-wise cold-pressing at pressures up to about 140,000 lbs./in.<sup>2</sup> to a specific gravity of 7.6 to 7.7, thereafter heating the mass for approximately one hour at about 850° to 900° C., and then rapidly quenching the same.

9. Process according to claim 1, wherein the mass is

quenched after the reheating, and then is soaked at a temperature below the transformation point.

10. Process according to claim 6, wherein the mass, after the quenching, is soaked at a temperature of about 650° C.

11. Process according to claim 8, wherein the mass, after the quenching, is soaked at a temperature of about 650° C.

## References Cited in the file of this patent

## UNITED STATES PATENTS

2,491,238 Whitney ----- Dec. 13, 1949  
5 2,741,827 Koehler ----- Apr. 17, 1956